

Feb. 2, 1937.

H. A. SCHWARTZ

2,069,423

FERROUS ALLOY

Filed March 5, 1932



INVENTOR

HARRY A. SCHWARTZ

BY

Clarence Kerr

ATTORNEY

Patented Feb. 2, 1937

2,069,423

# UNITED STATES PATENT OFFICE

2,069,423

## FERROUS ALLOY

Harry A. Schwartz, Cleveland Heights, Ohio, assignor to National Malleable and Steel Castings Company, Cleveland, Ohio, a corporation of Ohio

Application March 5, 1932, Serial No. 596,971

9 Claims. (Cl. 75—123)

This invention relates to the manufacture of ferrous alloys, its principal objects being the production of an alloy of improved characteristics and the provision of an improved and simplified process of making malleable ferrous alloys.

I have found that in a ferrous alloy which contains substantially less carbon than that normally found in white iron for making malleable cast iron and which contains silicon in greater proportions than normally found in high carbon steels, and preferably in proportions greater than normally found in white iron for malleable cast iron, graphite is produced in the iron as it cools in the mold, which graphite is in the form of nodular or temper carbon and with no substantial amounts of flaky carbon. I have further found that such alloys may be annealed at a lower temperature and in less time than that required to anneal malleable cast iron. For example, in the production of my malleable ferrous alloy the high temperature portion of the annealing process usually applied in making malleable cast iron may be omitted and the ferrous alloy may be subjected merely to the second or low temperature portion of the usual annealing process and need not be subjected to temperatures above the critical point during the annealing step.

In describing my new ferrous alloy reference will be made to the diagram which illustrates the relative proportions of carbon and silicon normally found in cast iron and white iron for malleable iron and in my ferrous alloy, the abscissae and ordinates of the graph showing percentages by weights of carbon and silicon respectively. The letter A designates the range of carbon and silicon normally found in cast iron and the letter B designates that normally found in white iron for malleable cast iron, although in some rare instances malleable iron may have been made containing carbon and silicon in the range shown within the dotted line at C. The line D designates the approximate lower limit of eutectiferous alloys as between carbon, silicon and iron.

With a white iron of the proportions illustrated at B and C and the normal quantities of phosphorus (about .14 to .19%), manganese (.25 to .40%) and sulphur (about .05 to .11%) no graphite is formed in the mold and the cast white iron is normally subjected to an annealing step above its critical temperature after which it is subjected to an annealing step at a temperature under the critical temperature, usually for about 30 hours.

I have found that by selecting a carbon content ranging from about 1% to 1.6% at the low limit 55 for silicon and from about 1% to 1.3% at the high

limit for silicon and a silicon content ranging from about 1% to 4% as illustrated in the diagram at E, a ferrous alloy is produced which upon cooling in the mold will precipitate carbon in nodular form and which may be annealed simply by subjecting the alloy to an annealing step at a temperature below the critical temperature of the alloy. The temperature of annealing will vary somewhat with the silicon content, as, for example, for the higher silicon material a temperature near 1470° F. will be desirable; for the lower silicon materials the temperature may be as little as 1290° F. or 1340° F. With an alloy containing about 1.5 to 2% silicon the annealing step at a temperature below the critical temperature may be carried out in the usual time required for the second or low temperature annealing step used in producing malleable cast iron, i.e., about 30 hours. By increasing the silicon content this annealing time may be reduced while with a lower content of silicon a somewhat greater time of heating may be required. The time and temperature of the annealing may of course be varied, depending upon the characteristics desired and the annealing may even be omitted, particularly where the higher proportion of silicon is used and where it is desired to retain the particular properties of combined carbon unaltered. Also the completely annealed metal may be heat treated to recombine such portions of uncombined carbon within the limits of solubility as may be desired or the product may be treated by quenching below the critical point in order to obviate intergranular brittleness and improve its ductility. This latter quenching below the critical point will be particularly useful in my product where the silicon is very high.

Nodular carbon may also be formed in the mold when a higher content of silicon is used than the high limit shown in diagram E, although the intergranular brittleness after annealing will increase with such higher content of silicon. Where this is not objectionable or where the annealing step may be omitted, such higher silicon alloy may be used. With such an alloy it may be desirable to reduce the phosphorus content to avoid intergranular brittleness.

The impurities normally present in white iron may be present in my new alloy although I prefer to reduce the phosphorus and sulphur slightly, although the proportions of these impurities are not essential. It is desirable, however, to maintain a sulphur-manganese balance.

The following are specific examples of some of the alloys which I have found to contain nodular

carbon when allowed to solidify in the mold, the remainder of the alloy being iron:

|    | Carbon | Silicon | Manganese | Sulphur | Phosphorus |
|----|--------|---------|-----------|---------|------------|
| 5  | 1.40   | 1.06    | 0.50      | 0.045   | 0.03       |
| 10 | 1.30   | 1.5     |           |         |            |
| 15 | 1.30   | 2.21    |           |         |            |
| 20 | 1.24   | 2.58    |           |         |            |
| 25 | 1.20   | 2.93    |           |         |            |
| 30 | 1.16   | 3.12    | .46       |         |            |
| 35 | 1.09   | 3.0     | .18       |         |            |

The manganese in Examples 2 to 5 was within the range .50 to .46% and the sulphur and phosphorus in all the Examples 1 to 7 were approximately the same.

In preparing the metal according to the present invention, any suitable materials may be employed. For instance, a charge of wash metal, presumably containing about 3.75% carbon, rivet scrap containing presumably about .10% carbon and 50% ferro silicon in such proportions as will give after melting the desired quantities of carbon and silicon. The materials may then be melted in a furnace such as an electric or other suitable furnace with the addition of sufficient ferro manganese to give the desired quantity of manganese.

The melt may then be heated to approximately 3000° F. and poured in a fluid condition, for example at around 2700° F. as the metal enters the mold. Variations may, however, be made in the maximum temperature and in the pouring temperature but it is preferred to use a somewhat higher temperature than that ordinarily used in pouring white or gray iron. After pouring, it is preferred to cool the metal slowly in the mold or to transfer it without previous cooling below the annealing temperature into a furnace maintained at that temperature.

In my new alloy the graphite formed on freezing is in an unexpected form, being present as small, dense nodules instead of flakes and exists in an unexpectedly large quantity. For instance, I have found that some .45 to .52% of graphite may be present in the metal as cast in the form of nodules, the balance of the carbon being combined as pearlite, while in a metal formed from a melt containing 1.86% carbon and 1.36 to 1.65% silicon, only .10 to .13% of the carbon was converted to graphite and that in the form of flaky carbon.

I have found that where the material making up the melt is of a nongraphitic character, proportions of carbon and silicon may be chosen which approach the line D more closely than will be the case where graphitic materials enter into the charge, also where the charge contains graphitic materials more attention must be paid to higher pouring temperatures than where the charge is made entirely of nongraphitic material.

If, because of abnormal cooling rates or abnormal additional constituents, the location of line D of the diagram be displaced, corresponding displacements of the high carbon boundary of the area E can or must be made.

As indicated in the diagram, ordinary malleable iron is a eutectiferous alloy (as between carbon, silicon and iron) and the balance between carbon and silicon is somewhat critical. If too much silicon or too much carbon is present to give a proper balance, flaky graphite will be formed in the mold and the material cannot be used since no amount of annealing will convert the flaky graphite into the nodular form. If the carbon or

silicon is balanced, cementite will be formed in such alloys which requires high temperatures for its speedy graphitization.

My new alloy is a non-eutectiferous alloy and, while it is necessary to maintain a certain degree of balance between carbon and silicon, it is a balance which is not nearly so sensitive, as illustrated in the diagram. With these non-eutectiferous alloys, the graphite separates in the mold in the form of nodules rather than as graphitic flakes.

It is not intended to restrict the invention to the particular alloys described since other low carbon alloys containing no element deleteriously affecting graphitization may be used as the starting point of my process. For example, some proportion of nickel, aluminum, titanium, zirconium or uranium might be substituted for a portion of the silicon in the low carbon irons referred to above, or such elements as molybdenum and copper may be added for their beneficial effect upon physical properties. Also, certain advantages of the invention may be utilized by using carbon and silicon in ratios somewhat outside the range indicated at E in the diagram. For example, I have found that an iron alloy containing 1.41% carbon, 3.08% silicon and .16% manganese when solidified in the mold did not contain either nodular carbon or flaky graphite but could be annealed at temperatures below the critical temperature and in less than six hours, although obviously the time was longer than it would have been if the proeutectoid carbon had been separated in the nodular form in the mold.

While I have shown the area E on the diagram bounded by 1.0% carbon, it should be understood that carbon contents as low as .75% may be used, although for practical reasons I prefer to work with this element above 1.0%.

The terms and expressions which have been employed are used as terms of description and not of limitation, and there is no intention, in the use of such terms and expressions, of excluding any equivalents of the features shown and described, or portions thereof, but it is recognized that various modifications are possible within the scope of the invention claimed.

I claim:

1. An alloy of iron containing about 1.0%–1.5% carbon, more than 2% to about 4% silicon and the balance being substantially all iron, about one-third of said carbon being present in nodular form.

2. An alloy of iron capable of being annealed below the critical temperature, said alloy containing about 1.0%–1.5% carbon, more than 2% to about 3.5% silicon and the balance being substantially all iron, about one-third of said carbon being present in nodular form, without substantial flake graphite.

3. An unannealed ferrous alloy containing graphitic carbon substantially entirely in the form of nodules and having a total carbon content of about 1% to 1.5% and a silicon content of more than 2 to about 4%, the balance being substantially all iron.

4. A ferrous alloy containing more than 2 to about 4% silicon and carbon ranging from 1% to 1.5% for the low limit of silicon to 1%–1.3% for the high limit of silicon, substantially the remainder of the alloy being iron.

5. A ferrous alloy containing more than 2 to about 3% of silicon and about 1.2–1.4% of carbon and the remainder being substantially iron.

6. A ferrous alloy containing silicon and car-

bon within the proportions defined by about 1 to 4% of silicon, 1 to 1.6% of carbon for the low range of silicon and 1 to 1.4% of carbon for the high range of silicon, together with .18% to less than .38% of manganese, the balance being substantially all iron.

5 7. A ferrous alloy containing 1.5 to 2% of silicon, 1 to 1.5% of carbon, .18 to less than .38% of manganese and the balance being substantially all iron.

10 8. A ferrous alloy containing carbon and silicon in proportions such as to give a non-eutectiferous

alloy and ranging from more than 2 to about 4% of silicon and about 1 to 1.6% of carbon, and substantially all the remainder of iron.

9. A ferrous alloy containing carbon and silicon in proportions such as to give a non-eutectic- 5 ferous alloy and ranging from above 1, to about 4% of silicon and about 1 to 1.6% of carbon, together with manganese in the proportion of about .18 to less than .38%, and substantially all the remainder of iron.

10

HARRY A. SCHWARTZ.